

## UNITED STATES PATENT OFFICE

ROLAND STERNER-RAINER, OF NECKARSULM, GERMANY, ASSIGNOR TO AMERICAN LURGI CORPORATION, OF NEW YORK, N. Y., A CORPORATION OF NEW YORK

## NONCORROSIVE ALUMINUM ALLOY

No Drawing. Application filed February 24, 1926, Serial No. 90,432, and in Switzerland December 17, 1925.

The present invention relates to aluminum alloys resistant to the action of corrosive agents and particularly to sea-water and to the production of such alloys.

5 It is well known that the alloys of aluminum and magnesium hitherto available are very deficient in resistance to the corrosive action of air, water and weather, and for this reason they have not been put to the extensive 10 use which their advantageous mechanical properties would otherwise have indicated.

It has now been found, however, that certain aluminum-magnesium alloys may be made, suitable for uses where corrosion-resisting properties are required, by means of 15 suitable treatment hereinafter more fully described.

The treatment of the magnesium-aluminum 20 alloys to render the corrosion-resistant 25 comprises a suitable thermal treatment advantageously in conjunction with suitable additions to the alloy.

The effect of the thermal treatment of the 25 invention in increasing the resistance of the alloys to corrosion is related to the fact that, in the presence of corrosive agents, potential differences arise between the dissimilar crystals of heterogeneous alloys, that is to say, of alloys made up, in the solid state, of 30 crystals of more than one physical type. These potential differences give rise to inter-crystalline electrolytic action and greatly accelerate corrosion.

Scientific research has shown that at ordinary 35 temperatures aluminum can hold magnesium in solid solution to the extent of about 10%. However, the casting of an aluminum alloy containing up to 10% magnesium does not result in castings of homogeneous crystal structure as might be expected. On the contrary, due to the high crystallization speed of the intermetallic compound  $Al_3Mg_2$  (containing over 37% magnesium), and to the low rate of diffusion, segregation occurs and structures of poor resistance to corrosion are formed. The high rate of crystallization results in the first crystals being of higher magnesium content than can be held in solid solution at ordinary temperatures. Since these 40 first  $\beta$ -type crystals are richer in magnesium

than the alloys as a whole, the latter  $\alpha$ -type crystals are deficient in magnesium. The resulting casting, therefore, comprises crystals of two different crystalline types and is accordingly deficient in resistance to corrosion 55 for the reasons noted above.

It has been found that the above described segregation of  $Al_3Mg_2$ , that is  $\beta$ -type crystals rich in magnesium, may be accomplished by subjecting the alloys to a temperature at 60 which the rate of diffusion of the magnesium, or of the intermetallic magnesium compound, is high, for a time sufficient to permit of substantially complete diffusion. In this way 65 there is produced a magnesium-aluminum alloy free from intercrystalline potential differences and of surprising resistance to corrosive agents.

For instance, magnesium-aluminum alloys containing 10% of magnesium may be held 70 for about an hour at a temperature of about 420° C. Under these conditions the excess magnesium in the  $\beta$ -type crystals diffuses into the magnesium-poor  $\alpha$ -type crystals, the  $\beta$ -type crystals being thereby transformed 75 into  $\alpha$ -type crystals so that the resulting alloy consists entirely of crystals of the same crystal-structure between which there is substantially no potential difference.

A similar result is obtained if the casting is 80 caused to cool down from a temperature of about 420° C. over a period of 5 to 8 hours.

A 5 to 20% solution of chromic acid is a valuable etching reagent for the determination 85 of the presence of the diverse crystal types and for following the diffusion and homogenizing of the structure of the alloy.

Of further value in increasing the resistance to corrosion of alloys of this type is 90 the addition to the alloys of substances which tend to produce protective oxide coatings or films on the surface of the alloy in contact with the air.

It has been found that antimony, bismuth 95 and cadmium answer the requirements above set forth and form highly suitable addition agents, either alone or in admixture, in aluminum alloys of the type under consideration.

However, the very low solubility of the above-named addition substances prevents their addition in more than very small amounts in order to avoid heterogeneity of crystal structure. These small amounts are ineffective to bring about an essential increase in the hardness or solidity of the alloy such as is desirable in many cases.

It has been found that the addition of metals of the iron group, such as manganese, nickel, etc., not only improves the mechanical properties of the alloys, without giving rise to intercrystalline potential differences in the alloys, but also increases the amount of the corrosion-reducing substances, such as 10 antimony, bismuth, and cadmium, which may be added without causing a substantial intercrystalline potential difference in the alloys.

An alloy composition within the scope of 15 the present invention is:

|                     |          |
|---------------------|----------|
| Magnesium           | 3 to 6%  |
| Manganese           | 1 to 4%  |
| Antimony            | up to 1% |
| Remainder aluminum. |          |

When the chromium is added to the alloys it should not be in amounts greater than 2%, and preferably less than 1%, because of its 20 effect in raising the solidification temperature of the alloys. For instance, with 2% chromium solidification begins at about 800°, with 3% chromium at about 900°, and with 4% chromium at about 1000°.

35 It is not necessary that all of the above mentioned types of addition substances be present in the alloys, as, for instance, magnesium-manganese-aluminum alloys, when produced according to the teachings of the 40 present invention, afford very considerable advantages over hitherto known aluminum alloys. The same is true when, instead of manganese or magnesium, small quantities of antimony, bismuth, or cadmium enter into 45 the composition of the alloy.

Further alloy compositions included within the scope of the present invention comprise:

|                       |         |
|-----------------------|---------|
| 50 1. Magnesium       | 3 to 6% |
| Manganese             | 1 to 4% |
| Chromium              | 0.5%    |
| Remainder aluminum    |         |
| 2. Magnesium          | 3 to 6% |
| 55 Cadmium            | 1.5%    |
| Remainder aluminum    |         |
| 3. Manganese          | 2%      |
| Chromium              | 0.5%    |
| 50 Antimony           | 3%      |
| 60 Remainder aluminum |         |

In the following claims the term "metal of the iron group" is intended to include manganese which, although it is not included 65 in group 8 of the Periodic System, performs

the same function in this invention as the metals of the iron group proper.

I claim:

1. A process of making corrosion-resistant alloys, which comprises subjecting an alloy of aluminum and magnesium containing not more than about 10 per cent of magnesium to an elevated temperature below its melting point until the alloy contains substantially only one crystal type. 70

2. A process of making corrosion-resistant alloys, which comprises subjecting an alloy of aluminum and magnesium containing not more than about 10 per cent of magnesium to a temperature of about 420° C. until the 80 alloy contains substantially only one crystal type.

3. A process of making corrosion-resistant alloys, which comprises subjecting an alloy of aluminum and magnesium containing not 85 more than about 10 per cent of magnesium at a temperature until the  $\beta$  crystals have disappeared.

4. A corrosion-resistant alloy of aluminum and magnesium, the magnesium content of 90 which does not substantially exceed the solid solubility of magnesium in aluminum, said alloy being free from magnesium-rich  $\beta$ -type crystals.

5. A corrosion-resistant alloy of aluminum 95 and magnesium containing not more than about 10% of magnesium and being free from magnesium-rich  $\beta$ -type crystals.

6. A corrosion-resistant alloy of aluminum and magnesium, the magnesium content of 100 which does not substantially exceed the solid solubility of magnesium in aluminum, said alloy being free from magnesium-rich  $\beta$ -type crystals and containing at least one metal of the group comprising antimony, bismuth and 105 cadmium.

7. A corrosion-resistant alloy of aluminum and magnesium, the magnesium content of 110 which does not substantially exceed the solid solubility of magnesium in aluminum, said alloy being free from magnesium-rich  $\beta$ -type crystals and containing at least one metal of the group comprising antimony, bismuth and 115 cadmium, and at least one metal of the iron group.

8. A corrosion-resistant alloy of aluminum and magnesium, the magnesium content of 120 which does not substantially exceed the solid solubility of magnesium in aluminum, said alloy being free from magnesium-rich  $\beta$ -type crystals and containing antimony.

9. A corrosion-resistant alloy of aluminum and magnesium, the magnesium content of 125 which does not substantially exceed the solid solubility of magnesium in aluminum, said alloy being free from magnesium-rich  $\beta$ -type crystals and containing antimony and manganese.

10. A corrosion-resistant alloy of aluminum 130 and magnesium, the magnesium content

of which does not substantially exceed the solid solubility of magnesium in aluminum, said alloy being free from magnesium-rich  $\beta$ -type crystals and containing up to 5% of 5 antimony and up to 8% of manganese.

In testimony whereof I affix my signature.

ROLAND STERNER-RAINER.

10

15

20

25

30

35

40

45

50

55